

## UNITED STATES PATENT OFFICE

2,346,635

## CORROSION INHIBITOR

Arthur C. Pabst, Douglaston, and John H. Prall,  
Lynbrook, N. Y., assignors to Socony-Vacuum  
Oil Company, Incorporated, a corporation of  
New York

No Drawing. Application April 28, 1942,  
Serial No. 440,888

22 Claims. (Cl. 252—73)

This invention relates to a corrosion inhibitor adapted to materially reduce the corrosive effect of aqueous liquids on metallic surfaces.

For many purposes aqueous liquids are maintained or circulated in contact with metallic surfaces. Serious problems of surface corrosion and/or formation of scale are almost universally met within such cases and provision is generally made to reduce these effects as much as possible. Among the varied uses of aqueous liquids to which this invention is applicable, the circulation of water in the cooling systems of internal combustion engines is important and may be taken here as typical.

All commercial anti-freezes used in automobile cooling systems are aqueous solutions having freezing points sufficiently low to assure a full flow of the cooling medium under normal pumping or thermo siphoning conditions. The most common anti-freezes are mono-, di- and poly-basic alcohols, such as methyl, ethyl, isopropyl alcohols, ethylene glycol and glycerine mixed with water in such proportions as to produce the required freezing point depression. Aqueous solutions of inorganic salts are less widely used.

Considerable aeration of the coolant in the automobile cooling systems takes place because of the high velocity of circulation and shaking of the automobile in motion. The aeration contributes to the rapid rate of oxidation of alcohols, which in turn produces acidic materials corrosive to the metals. The difficulty in finding adequate corrosion protection in automobile cooling systems lies in the variety of metals and alloys which come in contact with the coolant. Iron, brass, solder, aluminum and copper are the most commonly encountered metals. Some inhibitors, for instance, are specific in protecting aluminum but do not exert the same action on iron, and vice versa. Experience has shown that soluble mineral oils containing a sulfonate and soap emulsifier and nitrates represent about the best previously known all-purpose inhibitors for cooling systems containing a variety of metals.

We have discovered that nitrated fats represent a new group of materials admirably suited for the protection of multi-metal cooling systems. We have also discovered that nitrated fats are excellent inhibitors in water conditioning by which we mean a treatment of water for making it non-corrosive to the metal parts and free from deposition of scale. Water conditioning is most commonly applied to water circulated in steel, cast iron and aluminum, other metals being encountered in the adjunct pumping equipment.

Nitrated fats, including methods for preparation and their effects as lubrication assistants, are discussed in U. S. Patent No. 2,196,101, is-

sued April 12, 1940 to Carmichael, De Gray and Prall. It is there shown that superior results are obtained by using a composition of mineral lubricating oil containing tallow nitrated to an iodine number of about 30 or equivalent nitrated fat of other nature. For the present purposes, the fat is preferably nitrated to a somewhat greater degree, good results with nitrated tallow being obtained when the treated fat has an iodine number of about 5 to 35, while preferred compositions have an iodine number of about 18. In general, the nitration should be sufficient to improve alcohol solubility of the fat, and to render it water dispersible. The method of nitration described in the above patent are applicable to the present invention, it being necessary, of course, to increase the proportion of nitric acid to raw fat in order to obtain the desired, more extensive nitration.

20

## EXAMPLE I

## Preparation of anti-freeze

0.5 per cent of nitrated tallow (18 I. N.) is dissolved in an alcohol blend consisting of 60% methyl alcohol and 40% isopropyl alcohol. For charging into an automobile cooling system, this mixture is further diluted with water using one part of inhibited alcohol blend and three parts of water.

30

## EXAMPLE II

## Preparation of a water conditioner

|                           | Per cent<br>by weight |
|---------------------------|-----------------------|
| Nitrated tallow 18 I. N.— | 10                    |
| Sodium oleate—            | 3                     |
| Borax—                    | 1                     |
| Water—                    | 86                    |
| Total—                    | 100                   |

40

45

Nitrated tallow and soap are melted and dissolved in a portion of hot water, borax is dissolved in the balance of water, and the two solutions are combined into the finished product.

1.5 per cent of the above composition is sufficient to inhibit average New York city tap water. This amounts to 0.15% of nitrated tallow on the coolant. A correspondingly higher per cent of water conditioner may be necessary for harder water as is common practice with any water conditioner.

The efficacy of corrosion inhibitors for aqueous liquids can be readily demonstrated by experiments closely simulating the operating conditions in a cooling system of an internal combustion engine. This test, while not published and recognized by technical societies such as A. S. T. M., has received wide acceptance by the industry, particularly in the evaluation of

55

50

60

various water conditioners, hydraulic fluids and corrosion inhibitors. In this test, stainless steel racks holding test strips with metals usually encountered in cooling system, are half submerged in the liquid under test and refluxed for a period of 144 hours at 160° F. Upon completion of the test, the test strips are subjected to a standard procedure for removal of any traces of the product under test. The milligrams of metal lost, are a measure of the corrosiveness to any particular metal. The metals used in this test are as follows:

Cast iron (from an automobile cylinder head of a particular make)

Aluminum alloy (from an automobile cylinder head of a particular make)

Copper

Brass

Solder

It is known to those familiar with the art that cast iron and aluminum are the most vulnerable items in the series of metals listed above.

The value of nitrated fats is illustrated by data given below comparing nitrated tallow with a commercial inhibitor known as "Hydrotone" which is an aqueous solution of chromates, borax and meta-silicates.

Fats, including both solid fats and fatty oils, in general, are suitable for the purposes of the invention when nitrated at least to the point where corrosion inhibiting properties are developed to a substantial extent. Preferably those fats having a relatively high iodine number are employed. This general class of inhibitors is capable of being dispersed in aqueous liquids generally encountered, including aqueous solutions of alcohols used in aqueous cooling media to reduce the freezing point. The proportion of nitrated fat is, as might be expected, dependent to a large extent on the nature of the aqueous liquid. Amounts from about 0.05% to 25% by weight are effective but for most purposes, about 0.1% to about 5% of the inhibitor is used. In making up inhibited anti-freeze solutions, a comparable quantity of nitrated fat is used to provide the desired concentration upon dilution with water which is usually on the order of 1 part anti-freeze to 3 parts of water. In general, anti-freezes according to the invention will contain about 0.2% to about 20% of nitrated fat and the balance alcohol.

25 We claim:

1. An aqueous heat exchange liquid comprising a major proportion of water and a minor proportion of a water dispersible nitrated fat

| Water                    | Inhibitor used                                                          | Metal loss, mgms. |               |        |       |        |
|--------------------------|-------------------------------------------------------------------------|-------------------|---------------|--------|-------|--------|
|                          |                                                                         | Iron              | Alumi-<br>num | Solder | Brass | Copper |
| 1-100% N. Y. C. tap..... | 6 cc. hydrotone in 500 cc. of water.....                                | -108.7            | -27.0         | -7.0   | +0.4  | +0.4   |
| 2-100% N. Y. C. tap..... | 1.5% water conditioner containing 10% nitrated tallow (see Example 1D). | +1.1              | -2.5          | -1.6   | +0.4  | -0.6   |
| 3-100% N. Y. C. tap..... |                                                                         | -5.0              | -0.2          | -6.2   | -5.2  | -2.1   |

Nitrated fats show corrosion prevention effect on multi-metal systems when alcohol-water blends are used as coolants.

sufficient to substantially inhibit corrosion of metals by said liquid.

2. An aqueous heat exchange liquid comprising

| Water                   | Alcohol<br>blend by<br>volume | Inhibitor used              | Metal loss, mgms. |               |        |       |        |
|-------------------------|-------------------------------|-----------------------------|-------------------|---------------|--------|-------|--------|
|                         |                               |                             | Iron              | Alumi-<br>num | Solder | Brass | Copper |
| 4-75% N. Y. C. tap..... | 25                            | None.....                   | -76.2             | -6.9          | -0.8   | None  | -0.9   |
| 5-75% N. Y. C. tap..... | 25                            | 0.5% nitrated tallow.....   | -0.3              | -2.0          | -5.8   | -1.9  | -2.0   |
| 6-75% N. Y. C. tap..... | 25                            | Commercial preparation..... | -0.8              | -1.2          | -10.0  | -0.6  | -0.3   |

The last line is representative of present commercial antifreeze preparations being an inhibited product well received by the trade as an automobile anti-freeze. It will be seen that the nitrated tallow is on a par with the inhibitors in a satisfactory anti-freeze which is shown to contain an emulsified light oil and borax.

The following experiments prove that neither the fat alone nor the nitro group in combination with another organic radical is effective as a corrosion inhibitor.

a major proportion of water and a minor proportion of a water dispersible nitrated tallow sufficient to substantially inhibit corrosion of metals by said liquid.

55 3. An aqueous heat exchange liquid comprising a major proportion of water and a minor proportion of a water dispersible nitrated tallow having an iodine number of about 5 to 35 sufficient to substantially inhibit corrosion of metals by said liquid.

60 4. An aqueous heat exchange liquid comprising

| Water                   | Alcohol<br>blend by<br>volume | Inhibitor used          | Metal loss, mgms. |               |        |       |        |
|-------------------------|-------------------------------|-------------------------|-------------------|---------------|--------|-------|--------|
|                         |                               |                         | Iron              | Alumi-<br>num | Solder | Brass | Copper |
| 7-75% N. Y. C. tap..... | 25                            | 0.5% common tallow..... | -81.1             | -8.8          | -1.5   | -0.2  | -0.5   |
| 8-75% N. Y. C. tap..... | 25                            | 0.5% nitrobenzene.....  | -14.9             | 10.7          | -2.4   | -0.4  | -0.6   |

- a major proportion of water and about 0.15% of a water dispersible nitrated fat.
5. An aqueous heat exchange liquid comprising a major proportion of water and about 0.5% of a water dispersible nitrated fat.
6. An aqueous heat exchange liquid comprising a major proportion of water and about 0.05% to about 25% of a water dispersible nitrated fat.
7. An aqueous heat exchange liquid comprising a major proportion of water and about 0.1% to 10 about 5% of a water dispersible nitrated fat.
8. An aqueous heat exchange liquid comprising a major proportion of water, a substantial proportion of alcohol and a minor proportion of a water dispersible nitrated fat sufficient to substantially inhibit corrosion of metals by said liquid.
9. An aqueous heat exchange liquid comprising a major proportion of water, a substantial proportion of alcohol and a minor proportion of a water dispersible nitrated tallow sufficient to substantially inhibit corrosion of metals by said liquid. 20
10. An aqueous heat exchange liquid comprising a major proportion of water, a substantial proportion of alcohol and a minor proportion of a water dispersible nitrated tallow having an iodine number about 5 to 35 sufficient to substantially inhibit corrosion of metals by said liquid. 25
11. An aqueous liquid comprising a major proportion of water, a substantial proportion of alcohol and about 0.15% of a water dispersible nitrated fat.
12. An aqueous liquid comprising a major proportion of water, a substantial proportion of alcohol and about 0.5% of a water dispersible nitrated fat. 30
13. An aqueous heat exchange liquid comprising a major proportion of water, a substantial proportion of alcohol and about 0.05% to about 40 25% of a water dispersible nitrated fat.
14. An aqueous liquid comprising a major proportion of water, a substantial proportion of alcohol and about 0.1% to about 5% of a water dispersible nitrated fat.
15. An anti-freeze intended for dilution with water comprising a major proportion of a freezing point depressant and about 0.2% to about 20% of a water dispersible nitrated fat.
16. An anti-freeze intended for dilution with water comprising a major proportion of alcohol and about 0.2% to about 20% of a water dispersible nitrated fat.
17. An anti-freeze intended for dilution with water comprising a major proportion of a freezing point depressant and about 0.5% of a water dispersible nitrated fat. 15
18. An anti-freeze intended for dilution with water comprising a major proportion of alcohol and about 0.5% of a water dispersible nitrated fat.
19. An anti-freeze intended for dilution with water comprising a major proportion of a freezing point depressant and about 0.2% to about 20% of a water dispersible nitrated tallow.
20. An anti-freeze intended for dilution with water comprising a major proportion of alcohol and about 0.2% to about 20% of a water dispersible nitrated tallow.
21. An anti-freeze intended for dilution with water comprising a major proportion of a freezing point depressant and about 0.2% to about 20% of a water dispersible nitrated fat having an iodine number between about 5 and about 35.
22. An anti-freeze intended for dilution with water comprising a major proportion of a freezing point depressant and about 0.2% to about 20% of a water dispersible nitrated fat having an iodine number about 18. 35

ARTHUR C. PABST.  
JOHN H. PRALL.